

## UNITED STATES PATENT OFFICE

2,577,732

## PROCESS OF SPINNING VISCOSE

Rudolph S. Bley, Milligan College, Tenn., assignor  
to North American Rayon Corporation, New  
York, N. Y., a corporation of Delaware

No Drawing. Application November 16, 1950,  
Serial No. 196,086

18 Claims. (Cl. 18—54)

1

In the manufacture and production of continuous or discontinuous multi-filament threads and yarn of relatively high tenacity from viscose, a viscose solution is extruded through the fine ori-fices of a spinneret into a coagulating bath containing sulphuric acid, zinc sulphate, and sodium sulphate, to form partially coagulated viscose filaments therein. The partially coagulated (partially regenerated) filaments are then immediately stretched while passing them through a dilute acid bath which contains less acid and salts than the aforesaid coagulating bath, and this second bath is maintained at a temperature above 60° C. This so-called "hot water" spinning process, for example, is clearly disclosed in U. S. Patent No. 2,192,074, issued to Givens et al. on February 27, 1940, and the present invention constitutes a carrying forward of this prior art process.

Although it has been found that the Givens et al. process yields high quality products, nevertheless great difficulties are experienced in practising the same due to the formation of hard zinc sulphide deposits on the walls of the troughs containing the hot dilute acid bath and on the guide rollers submerged therein. Furthermore the aforesaid zinc sulphide deposits cause clogging of the pipe lines through which the coagulating bath is recirculated for reasons of economy. Since the hard deposits on the guide rollers are especially detrimental due to their tendency to cut the filaments led thereover during their bath travel, it becomes necessary to resort to frequent cleaning and replacement of the guide rollers to counteract this serious trouble.

Investigation has shown that zinc sulphide deposits are formed by chemical interaction of zinc sulphate in the dilute coagulating bath with hydrogen sulphide originating from the partially regenerated cellulose xanthate, and that this zinc sulphide formation can be minimized by decomposing (oxidizing) the hydrogen sulphide in statu nascendi by means of oxidizing anions, preferably persulphate anions introduced into the dilute coagulating bath through which the partially coagulated thread travels while being stretched. The persulphate anions are introduced into the hot, dilute coagulating bath by dissolving a suitable metal persulphate, for example sodium persulphate, potassium persulphate, ammonium persulphate, and other persulphates capable of forming soluble compounds in the presence of sulphuric acid and having a sufficient stability therein at a temperature of above 60° C. Ammonium persulphate is preferred for

2

reasons of economy. Sodium persulphate may be prepared from sodium sulphate, crystallized from waste spin bath, by well known electrolytic means, and used in this process.

5 Although in accordance with the present invention it is preferred to use persulphuric acid and soluble persulphates as oxidizing agents for reasons of efficiency and economy, nevertheless these particular chemicals can be replaced by 10 other water-soluble oxidizing agents, namely inorganic and organic per acids and water-soluble salts thereof, such as for example, peroxides, perborates, perchlorates, persilicates, percarbonates, permanganates, etc. Hypohalous acids 15 and water-soluble salts thereof, such as metal chlorites, bromites and iodites may serve also as suitable oxidizing agents for hydrogen sulphide and other unstable sulphur compounds produced during the regeneration of cellulose from cellulose xanthate (viscose). Since such sulphur compounds are oxidized in statu nascendi within the partially regenerated viscose filaments, fibers, films, etc., a considerable acceleration of the rate 20 of regeneration of cellulose from viscose (cellulose xanthate) is obtained inherently by using this novel spinning process in addition to the inhibition of zinc sulphide deposits as set forth above. Obviously, the thread may be advanced through the succeeding spin baths in a straight 25 or deviated path, or in the form of a helix having a plurality of loosely or closely spaced turns by means of suitable thread-storage, thread-advancing devices well known in the art of rayon manufacture, and by oxidizing the hydrogen sulphide 30 in the primary and/or secondary hot bath, zinc sulphide deposits which would normally be formed on the walls of the tanks and the thread-advancing devices are inhibited. The viscose used for the production of relatively high tenacity 35 yarn is prepared conventionally from rayon pulp containing more than 95% alpha cellulose and about 0.1 to 0.6% lignin.

40 The aforesaid oxidizing agents react with hydrogen sulphide to form negatively charged, colloidal sulphur, and this sulphur does not form dense deposits on the walls of the spin bath troughs, the guide rollers, or in the pipe lines. Moreover, the colloidal sulphur can be prevented 45 from settling on the aforesaid surfaces by the addition of anion-active compounds to the hot, dilute coagulating bath. The anion-active compounds enhance the negative charge of the colloidal sulphur particles and thus keep the same 50 in suspension. In other words, the colloidal sulphur particles are removed by "flootation." Any 55

anion-active compound may be used for this purpose provided it is sufficiently stable at temperatures above 60° C. Examples of suitable anion-active compounds are sulphonated high-molecular alcohol, sulphonated hydroxy benzenes having one or more straight chain alkyl groups having eight or more carbon atoms attached to the benzene nucleus, etc. such as soaps and products known commercially as aliphatic sulphonates, for example, sodium beta-oleylethanesulphonate, sodium beta-oleylamidoethanesulphonate, alkyl-aryl sodium sulphonates of the type R.Ar.SO<sub>3</sub>Na in which the long-chain alkyl group is derived from petroleum, and sulphates of long-chain alcohols prepared by the hydrogenation of fats. About .1 to .5 gram of an anion-active compound are generally sufficient per liter of bath to prevent the formation of loose sulphur deposits on the rollers submerged in the hot coagulating bath. The amount of persulphate ions to be provided in the hot coagulating bath depends upon the amount of hydrogen sulphide set free therein by the partially regenerated viscose filament, and can be readily determined by experiment. Generally speaking, about 3 grams per liter of bath are sufficient.

The primary acid coagulating bath contains sulphuric acid and also a sufficient amount of metallic sulphate to delay the decomposition of the viscose to cellulose hydrate. The metallic sulphate preferably employed is about 2.5 to 4% of zinc sulphate in addition to about 15 to 24% of sodium sulphate. The secondary, hot dilute acid coagulating bath contains less sulphuric acid and salts, and it is maintained at a temperature of at least 60° C., and it is preferable to employ a temperature of 80° C. or higher. The acid and salts for the dilute acid bath may be provided by acid and salts taken over by the filaments from the coagulating bath.

*Example*

A normal viscose solution was extruded through a spinneret into a coagulating bath containing about 9.5% of sulphuric acid, 17.3% sodium sulphate, 4.9% magnesium sulphate, 2.8% zinc sulphate, and 65.5% water (all percentages calculated on the weight of the bath), to form a 430 filament, 1100 denier yarn. The yarn bundle was stretched in a dilute acid bath containing about 2 grams per liter of sulphuric acid, .97 gram per liter of zinc sulphate, and a total salt content of about 6.7 grams per liter, to which about 3 grams of ammonium persulphate were added per liter. The hot, dilute coagulating bath was maintained at a temperature of 85° C. Only a loose sulphur deposit was formed on the rollers submerged in this bath, and this deposit was completely inhibited by dissolving .5 gram per liter of an anion-active compound (an alkylaryl sodium sulphonate of the type R.Ar.SO<sub>3</sub>Na in which the long-chain alkyl group is derived from petroleum) in the persulphate bath. The yarn had a dry strength of 2.95 grams per denier, a wet strength of 1.72 grams per denier, 15% dry elongation, and 18% wet elongation. Similar results were obtained following the example set forth in the Givens patent, No. 2,192,074, when persulphate ions were provided in the hot, dilute acid coagulating bath. The process may also be modified by adding a persulphate to the primary and/or the secondary coagulating baths. The spinning process may be carried out with any other oxidizing agent set forth above in lieu of ammonium persulphate.

The process may obviously be modified with-

out departing from the spirit and scope of the invention as set forth in the appended claims.

This application is a continuation-in-part of my application Serial No. 727,947 filed February 11, 1947, for Process of Spinning Viscose, now abandoned.

What is claimed is:

1. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing said dilute acid bath with a sufficient amount of a salt selected from the group consisting of ammonium persulphate, sodium persulphate and potassium persulphate to minimize the evolution of hydrogen sulphide therein, whereby the formation of zinc sulphide is inhibited.

2. In a process for the manufacture and production of continuous or discontinuous filaments of relatively high tenacity from viscose which includes partially regenerating the viscose filaments in a bath containing sulphuric acid and sodium sulphate and at least 2.5% of zinc sulphate, the proportion of the said salts to the acid being such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing said dilute acid bath with a sufficient amount of a salt selected from the group consisting of ammonium persulphate, sodium persulphate and potassium persulphate to minimize the evolution of hydrogen sulphide therein, whereby the formation of zinc sulphide is inhibited.

3. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing said dilute acid bath with a sufficient amount of a salt selected from the group consisting of ammonium persulphate, sodium persulphate and potassium persulphate to decompose the hydrogen sulphite evolved by said partially decomposed cellulose xanthate

filaments to form colloidal sulphur and with a sufficient amount of a dissolved anion-active compound to maintain said sulphur in suspension.

4. Process according to claim 1, in which the acid and salts for the dilute acid bath are being provided by acid and salts taken over by the filaments from the coagulating bath.

5. Process according to claim 2, in which the acid and salts for the dilute acid bath are being provided by acid and salts taken over by the filaments from the coagulating bath.

6. Process according to claim 3, in which the acid and salts for the dilute acid bath are being provided by acid and salts taken over by the filaments from the coagulating bath.

7. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially regenerated cellulose xanthate filaments, the improvement which comprises providing said dilute acid bath with a sufficient amount of ammonium persulphate to minimize the evolution of hydrogen sulphide therein, whereby the formation of zinc sulphide is inhibited.

8. In a process for the manufacture and production of continuous or discontinuous filaments of relatively high tenacity from viscose which includes partially regenerating the viscose filaments in a bath containing sulphuric acid and sodium sulphate and at least 2.5% of zinc sulphate, the proportion of said salts to the acid being such that immediate complete regeneration is prevented, then stretching the thus partially regenerated filaments with attendant reduction in cross section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing said dilute acid bath with a sufficient amount of ammonium persulphate to minimize the evolution of hydrogen sulphide therein, whereby the formation of zinc sulphide is inhibited.

9. In a process for the manufacture and production of continuous or discontinuous filaments of relatively high tenacity from viscose which includes partially regenerating the viscose filaments in a bath containing sulphuric acid and zinc and sodium sulphate wherein the proportion of the salts to the acid is such that immediate complete regeneration is prevented, then stretching the thus partially regenerated filaments, with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which com-

prises providing said dilute acid bath with a sufficient amount of ammonium persulphate to decompose the hydrogen sulphide evolved by said partially decomposed xanthate filaments to form colloidal sulphur and with a sufficient amount of a dissolved anion-active compound to maintain said sulphur in suspension.

10. A process according to claim 7, in which the acid and salts for the dilute acid bath are being provided by acid and salts taken over by the filaments from the coagulating bath.

11. A process according to claim 8, in which the acid and salts for the dilute acid bath are being provided by acid and salts taken over by the filaments from the coagulating bath.

12. A process according to claim 9, in which the acid and salts for the dilute acid bath are being provided by acid and salts taken over by the filaments from the coagulating bath.

13. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially regenerated cellulose xanthate filaments, the improvement which comprises providing said dilute acid bath with a sufficient amount of a metal persulphate to minimize the evolution of hydrogen sulphide therein, whereby the formation of zinc sulphide is inhibited, said persulphate being dissolved in said dilute acid and being sufficiently stable therein at a temperature of above 60° C.

14. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially regenerated cellulose xanthate filaments, the improvement which comprises providing said bath and said dilute acid bath with a sufficient amount of a metal persulphate to minimize the evolution of hydrogen sulphide therein, whereby the formation of zinc sulphide is inhibited, said persulphate being dissolved in said bath and said dilute acid bath and being sufficiently stable therein at a temperature of above 60° C.

15. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated fila-

ments with attendant reduction in cross-section and evolution of hydrogen sulphide while passing them through a dilute acid bath which contains less acid than the aforesaid bath and is maintained at a temperature above 60° C., which increases the plasticity of the partially regenerated cellulose xanthate filaments, the improvement which comprises providing said bath and said dilute acid bath with a sufficient amount of a persulphate selected from the group consisting of ammonium persulphate, sodium persulphate and potassium persulphate, whereby the formation of zinc sulphide is inhibited.

16. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus partially regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing at least one of said acid baths with a sufficient amount of an oxidizing agent to minimize the evolution of hydrogen sulphide therein, whereby the formation of zinc sulphide is inhibited, said oxidizing agent being dissolved in said bath.

17. In a process for the manufacture and production of continuous or discontinuous filaments of relatively high tenacity from viscose which includes partially regenerating the viscose filaments in a bath containing sulphuric acid and sodium sulphate and at least 2.5% of zinc sulphate, the proportion of the said salts to the acid being such that immediate complete re-

generation is prevented, then stretching the thus regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing at least one of said acid baths with a sufficient amount of an oxidizing agent to minimize the evolution of hydrogen sulphide therein, whereby the formation of zinc sulphide is inhibited, said oxidizing agent being dissolved in said bath.

18. In a process for the manufacture and production of continuous or discontinuous filaments of relatively high tenacity from viscose which includes partially regenerating the viscose filaments in a bath containing sulphuric acid and zinc and sodium sulphates wherein the proportion of the salts to the acid is such that immediate complete regeneration is prevented, then stretching the thus regenerated filaments with attendant reduction in cross-section and evolution of hydrogen sulphide while passing them through a dilute acid bath which contains less acid than the aforesaid bath and is maintained at a temperature above 60° C., which increases the plasticity of the partially decomposed cellulose xanthate filaments, the improvement which comprises providing at least one of said acid baths with a sufficient amount of an oxidizing agent to decompose the hydrogen sulphide evolved by said partially decomposed cellulose xanthate filaments to form colloidal sulphur and with a sufficient amount of an anion-active compound to maintain said sulphur in suspension, said oxidizing agent and said anion-active compound being dissolved in said bath.

RUDOLPH S. BLEY.

No references cited.